

## UNITED STATES PATENT OFFICE

2,206,946

## MANUFACTURE AND TREATMENT OF ORGANIC MATERIALS COMPRISING ORGANIC ESTERS

Henry Dreyfus, London, England

No Drawing. Application January 13, 1938, Serial No. 184,801. In Great Britain January 18, 1937

10 Claims.

(Cl. 8—130)

This invention relates to the saponification of threads, fibres, yarns, fabrics, ribbons, films and like materials having a basis of cellulose acetate or other organic ester of cellulose.

It is difficult to effect saponification, and particularly partial saponification of materials of the kind referred to above in such a way that the products have desirable tensile properties and at the same time can be dyed uniformly with cotton dyes without streakiness or similar defects.

I have now found that the desired results can readily be obtained by treating the materials in an alkaline saponifying bath formed by dissolving in an aqueous medium, two salts of a weak 15 polybasic acid with the same or different strong bases, said salts containing different molecular proportions of the acid radicle. Thus, for example, the bath may be made from mixtures of trisodium or potassium phosphate with disodium 20 or potassium phosphate, of sodium, potassium, calcium or barium sulphides with sodium, potassium, calcium or barium hydrosulphides, or of sodium or potassium carbonates with the corresponding bicarbonates. Preferably both salts 25 are of alkaline reaction. Salts of alkali metals are particularly suitable.

It is generally of advantage for the salt of lower acid radicle content to predominate considerably in the mixture. It may, for example, conveniently 30 be present to the extent of 5-10 or 15 times the molecular proportion of the salt of higher acid radicle content. The concentration in which the salts are employed will depend on the nature of the materials treated, the degree of saponification 35 desired and the alkalinity of the salts, i. e., the pH value of aqueous solutions of given concentration. When treating ordinary cellulose acetate yarn, for example having an acetyl value of between 51 and 54 so as to effect a reduction 40 in the acetyl content of between 20 and 30%, the bath may contain an amount of trisodium phosphate ranging from that theoretically required to produce the desired saponification to twice the theoretical amount together with some 45 8-15% on the weight of the trisodium phosphate of disodium hydrogen phosphate, the bath volume being between 50:1 and 80:1, e. g., 60:1 or 70:1. Similar proportions are suitable when the corresponding potassium salts are used or when sodium carbonate is used in admixture with sodium bicarbonate. When sodium or potassium sulphide is used in conjunction with the corresponding hydrosulphide, the concentration should preferably be reduced, i. e., a bath volume greater 55 than 60:1 should be used. With the corresponding calcium salts, however, the concentration should preferably be considerably higher, that is the amount of salts used should be several times that theoretically required and in addition the bath volume may be reduced, for example to 30:1.

The temperature of the bath may be relatively low, for example below 40 or 50° C., though it is preferable to carry out the saponification at considerably higher temperatures, for example from 60-80° C.

When the process is applied to materials which have been stretched considerably at some stage in their manufacture, for example in the course of a wet spinning operation or of a stretching operation carried out on threads after spinning while 10 they are under the action of an organic swelling agent or of steam or of hot water, it is of advantage to use baths of higher concentration than would be used, other things being equal, in the treatment of ordinary unstretched threads of the 15 same material. If, on the other hand, the threads treated have undergone a shrinking operation after stretching or without their having been stretched, low concentrations of the saponifying agent may be used.

The saponification may be carried out on the materials in any suitable form, for example in hank form or wound on to perforated bobbins or other package carriers. On the other hand the materials may be drawn continuously through the saponifying bath but as the saponification 20 baths of the invention are necessarily somewhat slow in action, continuous operation does not in general present advantages over saponification in package form.

The following examples illustrate the invention.

## Example 1

A bath for completely saponifying 100 lbs. of 35 cellulose acetate yarn is made up by dissolving 200 lbs. of trisodium phosphate and about 20 lbs. of disodium hydrogen phosphate in 600 gallons of water. The yarn is introduced in hank form and allowed to remain in the bath at a temperature 40 of 70-80° C. until saponification is complete.

Instead of treating the yarn in hank form, it may be any other suitable package form, for example wound on to foraminous bobbins. Fabrics of cellulose acetate can be treated in a similar way.

## Example 2

A bath is made up as described in Example 1, but using the following quantities for each 100 lbs. of yarn:

|                             |         |     |
|-----------------------------|---------|-----|
| Trisodium phosphate         | lbs.    | 100 |
| Disodium hydrogen phosphate | lbs.    | 15  |
| Water                       | gallons | 300 |

The yarn is allowed to remain in the bath at 55 80-90° C. until 20-30% of the original acetyl content is removed.

Though the invention has been described with particular reference to cellulose acetate materials, the process of the invention is also applicable to 60

the saponification of materials having a basis of other organic esters of cellulose, for example cellulose formate, propionate, butyrate, mixed esters such as cellulose nitrate-acetate, nitrate-propionate, acetate-propionate, acetate-propionate-nitrate and ether esters such as ethyl cellulose acetate and oxyethyl cellulose acetate.

The degree of saponification may be sufficient to reduce the acidyl content of the ester by 10 15-20% or even less. It is preferably somewhat higher however, for example sufficient to reduce the acidyl content by 20-25 or 30%. Considerably higher degrees of saponification may be obtained, sufficient to remove, for example 35 or 15 40-50% or even more of the acidyl content of the materials according to the particular purpose in view.

Having described my invention, what I desire to secure by Letters Patent is:

20 1. Process for the production of improved artificial materials, which comprises saponifying threads, fibres, yarns, fabrics, ribbons or like materials having a basis of organic ester of cellulose by treatment in an aqueous bath containing two alkali metal salts of the same weak inorganic polybasic acid, one of said salts containing a higher molecular proportion of acid radicle than the other and the bath being alkaline owing solely to hydrolysis of at least one of 25 said salts.

2. Process for the production of improved artificial materials which comprises saponifying threads, fibres, yarns, fabrics, ribbons or like materials having a basis of organic ester of cellulose by treatment in an aqueous bath containing two salts of the same alkali metal with the same weak inorganic polybasic acid, one of said salts containing a higher molecular proportion of acid radicle than the other and the bath 30 being alkaline owing solely to hydrolysis of at least one of said salts.

3. Process for the production of improved artificial materials which comprises saponifying threads, fibres, yarns, fabrics, ribbons or like 45 materials having a basis of organic ester of cellulose by treatment in an aqueous bath made by dissolving in an aqueous medium two salts of the same alkali metal with the same weak inorganic polybasic acid, one of said salts containing a higher molecular proportion of acid radicle than the other and the bath being alkaline owing solely to hydrolysis of at least one of said salts, the salt containing the lower molecular proportion of acid being present in excess.

55 4. Process for the production of improved artificial materials which comprises saponifying threads, fibres, yarns, fabrics, ribbons or like materials having a basis of organic ester of cellulose by treatment in an aqueous bath made 60 by dissolving in an aqueous medium two salts of the same alkali metal with the same weak inorganic polybasic acid, one of said salts containing a higher molecular proportion of acid radicle than the other and the bath being alkaline owing solely to hydrolysis of at least one of said salts, the salt containing the lower proportion of acid radicle being present in an amount ranging from that theoretically required to produce the desired saponification to twice that amount and the 65 salt containing the lower proportions of acid radicle being present to the extent of 5 to 15 times the molecular proportion of the salt of higher acid radicle content.

5. Process for the production of improved artificial materials which comprises saponifying threads, fibres, yarns, fabrics, ribbons or like materials having a basis of organic ester of cellulose by treatment in an aqueous bath made by 5 dissolving in an aqueous medium two salts of the same alkali metal with phosphoric acid, one of said salts containing a higher molecular proportion of acid radicle than the other and the bath being alkaline owing solely to hydrolysis of at least one of said salts, the salt containing the lower molecular proportion of acid being present in excess.

6. Process for the production of improved artificial materials which comprises saponifying threads, fibres, yarns, fabrics, ribbons or like materials having a basis of organic ester of cellulose by treatment in an aqueous bath made by dissolving in an aqueous medium two salts of the same alkali metal with carbonic acid, one of said salts containing a higher molecular proportion of acid radicle than the other and the bath being alkaline owing solely to hydrolysis of at least one of said salts, the salt containing the lower molecular proportion of acid being present in excess.

7. Process for the production of improved artificial materials which comprises saponifying threads, fibres, yarns, fabrics, ribbons or like materials having a basis of organic ester of cellulose by treatment in an aqueous bath made by dissolving in an aqueous medium trisodium phosphate and disodium hydrogen phosphate, the trisodium phosphate being in excess and the bath being alkaline solely owing to hydrolysis of one of the salts.

8. Process for the production of improved artificial materials which comprises saponifying threads, fibres, yarns, fabrics, ribbons or like materials having a basis of organic ester of cellulose by treatment in an aqueous bath made by dissolving in an aqueous medium trisodium phosphate and disodium hydrogen phosphate, the trisodium phosphate being present in an amount ranging from that theoretically required to produce the desired saponification to twice that amount and the trisodium phosphate being present to the extent of 5 to 15 times the molecular proportion of the disodium hydrogen phosphate.

9. Process for the production of improved artificial materials, which comprises saponifying threads, fibres, yarns, fabrics, ribbons or like materials having a basis of cellulose acetate by treatment in an aqueous bath containing two alkali metal salts of the same weak inorganic polybasic acid, one of said salts containing a higher molecular proportion of acid radicle than the other and the bath being alkaline owing solely to hydrolysis of at least one of said salts.

10. Process for the production of improved artificial materials which comprises saponifying threads, fibres, yarns, fabrics, ribbons or like materials having a basis of cellulose acetate by treatment in an aqueous bath made by dissolving in an aqueous medium two salts of the same alkali metal with carbonic acid, one of said salts containing a higher molecular proportion of acid radicle than the other and the bath being alkaline owing solely to hydrolysis of at least one of said salts, the salt containing the lower molecular proportion of acid being present in excess.